



US007122245B2

(12) **United States Patent**  
**Morton-Finger**

(10) **Patent No.:** **US 7,122,245 B2**  
(45) **Date of Patent:** **\*Oct. 17, 2006**

(54) **MULTI-LAYER MONOFILAMENT AND PROCESS FOR MANUFACTURING A MULTI-LAYER MONOFILAMENT**

(75) Inventor: **Jürgen Morton-Finger**, Weinheim (DE)

(73) Assignee: **Motech GmbH Technology & Systems**, Ober-Abtsteinach (DE)

(\*) Notice: Subject to any disclaimer, the term of this patent is extended or adjusted under 35 U.S.C. 154(b) by 0 days.

This patent is subject to a terminal disclaimer.

(21) Appl. No.: **10/772,162**

(22) Filed: **Feb. 3, 2004**

(65) **Prior Publication Data**

US 2004/0170830 A1 Sep. 2, 2004

(30) **Foreign Application Priority Data**

Feb. 20, 2003 (DE) 103 07 174

(51) **Int. Cl.**

**D01F 6/00** (2006.01)  
**D01F 8/00** (2006.01)

(52) **U.S. Cl.** 428/364; 428/370

(58) **Field of Classification Search** 428/364, 428/370

See application file for complete search history.

(56) **References Cited**

**U.S. PATENT DOCUMENTS**

3,616,130 A \* 10/1971 Rogosch et al. 428/110  
4,229,394 A \* 10/1980 Rasmussen 264/46.1  
5,071,705 A \* 12/1991 Tanaka et al. 428/370  
5,814,404 A \* 9/1998 Rutherford et al. 428/364

**OTHER PUBLICATIONS**

Dictionary of Fiber & Textile Technology, p. 99, date 1965-1990.\*

\* cited by examiner

*Primary Examiner*—N. Edwards

(74) *Attorney, Agent, or Firm*—Andrew Wilford

(57) **ABSTRACT**

A multi-layer monofilament consisting of multiple layers that are extruded simultaneously in a single process step, having a first layer made from plastic A, a second layer, which is bonded directly to the first layer, made from plastic b, and a third layer, which is bonded directly to the second layer, made from plastic C, plastic B being a bonding agent between the two plastics A and C.

**4 Claims, 3 Drawing Sheets**





FIG.1



FIG.2



FIG.3



**FIG. 4**

## 1

**MULTI-LAYER MONOFILAMENT AND  
PROCESS FOR MANUFACTURING A  
MULTI-LAYER MONOFILAMENT**

**FIELD OF THE INVENTION**

The invention relates to a multi-layer monofilament and, more particularly, to a method for manufacturing such a multi-layer monofilament and the monofilament made by that method.

**BACKGROUND OF THE INVENTION**

The principle of manufacturing or spinning two-layer monofilaments or bicomponent filaments from two different thermoplastic plastics is known. In this way, monofilaments receive corresponding properties, which cannot be achieved in one plastic alone.

It is known to produce these monofilaments from two layers either in a side-by-side arrangement or in a core/sheath arrangement. Many bicomponent filaments, particularly those with a core/sheath structure, have the disadvantage that the adhesion between the two layers (core and sheath) is inadequate and they can therefore easily delaminate. Particularly when these monofilaments are stretched, it often happens that the sheet layer peels away from the core like an onionskin. These problems occur in many plastic pairs.

**OBJECTS OF THE INVENTION**

An object of the invention is to provide an improved multi-layer monofilament of the type described at the outset which does not suffer from the problems explained above and in which the individual layers are adequately bonded with each other.

Another object of this invention is to provide a multilayer monofilament which resists delamination to a greater extent than has been the case heretofore and, in particular, is more stable than earlier laminated filaments.

It is also an object of this invention to provide a method of making a multilayer filament which has greater resistance to delamination.

**SUMMARY OF THE INVENTION**

These objects are achieved with a multi-layer monofilament consisting of multiple layers that are extruded or spun simultaneously in a single process step, having a first layer made from plastic A, a second layer, which is bonded directly to the first layer, made from plastic B, and a third layer, which is bonded directly to the second layer, made from plastic C, plastic B being a bonding agent between the two plastics A and C.

Multiple layers are said to be simultaneously extruded or spun in particular when the liquefied plastics intended for use in the multiple layers of the monofilament are ejected from the same spinning orifice or spinning device together, thereby creating the multi-layer monofilament. A spinning device of such kind is normally equipped with multiple spinning orifices.—For the purpose of the invention, a bonding agent is a plastic that serves to improve the adhesive bond between two plastics to be bonded.

The scope of the invention applies expressly to multiple-layer monofilaments including only three layers. Thus the filament of the invention is preferably a three-layer monofilament.

## 2

A highly advantageous embodiment, to which particular importance attaches within the scope of the invention, has a core/sheath structure, wherein the core of the monofilament is formed by plastic A, wherein this core is at least partly enclosed by the second layer consisting of plastic B, and wherein the second layer consisting of plastic B is at least partly enclosed by the third layer consisting of plastic C. In this core/sheath structure, the core consisting of plastic A is thus equivalent to the first layer consisting of plastic A. For practical reasons, the core has a circular or elliptical cross-section. The scope of the invention expressly includes the fact that the core is fully enclosed by the second layer consisting of plastic B, and that it preferably has a circular cross-section. According to a preferred embodiment, the second layer consisting of plastic B is entirely enclosed by the third layer consisting of plastic C and that it has a circular cross-section for practical purposes.

In all cases, the scope of the invention expressly includes the fact that a multi-layer monofilament according to the invention has a side-by-side structure.

According to one particularly preferred embodiment of the invention, plastic B, i.e. the adhesive agent, is an ethylene-vinylacetate copolymer and/or a methacrylate copolymer.

Preferably, one of the two layers to be bonded by means of plastic B, i.e. by means of the bonding agent, i.e. the first layer consisting of plastic A or the third layer consisting of layer C, is made from at least one plastic from the group which consists of polyethylene terephthalate (PET), polyamide (PA), polyamide copolymer, polypropylene (PP). The scope of the invention expressly includes the fact that a polyamide 6 and/or polyamide 6.6 and/or polyamide 6.12 is used as the polyamide. According to a preferred embodiment of the invention, the other of the two layers to be bonded by means of plastic B, i.e. by means of the bonding agent, i.e. the first layer consisting of plastic A or the third layer consisting of layer C is made from at least one plastic from the group which consists of polyethylene (PE), polyoxymethylene (POM), polyphenylene sulphide (PPS), polymethylmethacrylate (PMMA), polybutyl n terephthalate (PBT), polyvinyl chloride (PVC), polyether etherketone (PEEK), and polyethylene naphthalate (PEN).

In the process of the invention multi-layer monofilament is produced by means of a spinning device having a plurality of spinning orifices, wherein one liquefied plastic for each layer of the monofilament is directed to the respective spinning orifice and wherein the liquefied plastics for various layers are ejected from the spinning orifice together, thereby forming a single multi-layer monofilament.

According to a particularly preferred embodiment of the invention, a multi-layer monofilament having a core/sheath structure is produced, wherein the liquid plastic of plastic A is directed to each spinning orifice via a feeding channel provided centrally over the spinning orifice to form the core of the monofilament, wherein the liquefied plastic of plastic B (bonding agent) is directed to form an inner sheet via an inner feeding slit encircling the feeding channel in annular manner, and wherein the liquefied plastic of plastic C is directed to form an outer sheet via an outer feeding slit encircling the inner, annular feeding slit. The scope of the invention expressly provides for the fact that the inner and/or the outer feeding slits is/are feeding slits that encircle the feeding channel in annular manner.

According to a particularly preferred embodiment of the invention, the multi-layer monofilaments are stretched after

spinning. Stretching is advantageously done in one to three stages. Stretching may take place in air, or in steam or in water.

The multi-layer monofilaments are preferably fixed following the stretching. In this case, fixing means that the multi-layer monofilaments are heated, specifically to a temperature above 20° C., preferably above 25° C. Fixing may also take place in one to three stages and is preferably done in air or in steam or in water.

The multi-layer monofilaments are preferably fixed following the stretching. In this case, fixing means that the multi-layer monofilaments are heated, specifically to a temperature above 20° C., preferably above 25° C. Fixing may also take place in one to three stages and is preferably done in air or in steam or in water.

The invention is based on the realization that the layers of the multi-layer monofilaments according to the invention adhere to each other surprisingly strongly. When these multi-layer monofilaments are stretched, the layers do not delaminate. In addition, the multi-layer monofilaments according to the invention may be manufactured relatively simply and inexpensively.

#### BRIEF DESCRIPTION OF THE DRAWING

The above and other objects, features, and advantages will become more readily apparent from the following description, reference being made to the accompanying drawing in which:

FIG. 1 is a transverse cross section drawn to a greatly enlarged scale and diagrammatically showing a multilayer monofilament according to the invention;

FIG. 2 is a section through one orifice of a multiorifice spinning head for producing the monofilament of the invention

FIG. 3 is a diagram of an apparatus for producing monofilament in accordance with the principles of this invention; and

FIG. 4 is a section similar to FIG. 1 showing the side-by-side structure.

#### SPECIFIC DESCRIPTION

In the embodiment shown in FIG. 1, the multi-layer monofilament is formed as a three-layer monofilament specifically having a core/sheath structure. Core 1 here corresponds to the first layer of the multi-layer monofilament made from plastic A. Preferably and in the embodiment, core 1 has a circular cross-section. In the embodiment shown in this FIGURE, this core 1 is surrounded by an inner sheath 2, which corresponds to the second layer consisting of plastic B, i.e. the bonding agent. Inner sheath 2 surrounds core 1 in an annular manner. This inner sheath 2 is in turn surrounded by an outer sheath 3, which corresponds to the third layer consisting of plastic C. This outer sheath 3 surrounds inner sheath 2 consisting of plastic B in annular manner. In this embodiment, inner sheath 2 may consist of ethylene vinylacetate copolymer as a bonding agent.

In FIG. 2 I have shown a multiorifice spinning head 10, one orifice of which is visible at 11. As can be seen from FIG. 2, the orifice 11 is associated with guides 12 and 13 which define annular slits 14 and 15. The core synthetic resin, here seen at 16 passes through the guide 13 and is surrounded by the bonding plastic 17 which is applied through the annular slit 15 as an inner sheath to the core. The outer sheath, which is applied by the slit 14 to the intermediate layer is of the plastic 18 to which the bonding plastic 17 has an especial affinity.

As will be apparent from FIG. 3, the monofilament 20 from the multi orifice head 10 are subjected to stretching over rolls 21, 22, and 23 which are successively driven with greater peripheral speeds. The stretching is carried out in air, in steam or in water. After stretching, the monofilaments are fixed at 24 by heating in air, steam or water as has previously been described.

FIG. 4 is a view similar to FIG. 4 of a monofilament made from plastics A, B and C and wherein the layers 1', 2' and 3', corresponding to the sheaths and core of the embodiment of FIG. 1 are in a side by side relationship.

I claim:

1. A continuous multi-layer monofilament having a circular cross section and consisting of multiple layers that are extruded simultaneously in a single process step from a single spinning orifice, the monofilament having  
a first layer made from first plastic,  
a second layer bonded directly to the first layer, made from a second plastic that is an ethylene-vinylacetate copolymer or a methylacrylate copolymer, and  
a third layer bonded directly to the second layer and made from a third plastic, the second plastic being a bonding agent for bonding the first and third plastics, one of the first and third plastics being selected from the group which consists of polyethylene terephthalate (PET), polyamide (PA), polyamide copolymer, and polypropylene (PP), the other of the first and third plastics being selected from the group which consists of polyoxymethylene (POM), polyphenylene sulphide (PPS), polymethylmethacrylate (PMMA), polybutylene terephthalate (PBT), polyvinyl chloride (PVC), polyether etherketone (PEEK), and polyethylene naphthalate (PEN).

2. The multi-layer monofilament according to claim 1 wherein the monofilament consists of three layers.

3. The multi-layer monofilament according to claim 1 wherein the monofilament has a core/sheath structure, that the core of the monofilament is formed by the first plastic, the core is at least partly enclosed by the second layer consisting of the second plastic, and the second layer consisting of the second plastic is at least partly enclosed by the third layer consisting of the third plastic.

4. The multi-layer monofilament according to claim 1 wherein the monofilament has a side-by-side structure.